

# UNITED STATES PATENT OFFICE.

FREDERICK M. BECKET, OF NIAGARA FALLS, NEW YORK, ASSIGNOR TO ELECTRO METALLURGICAL COMPANY, OF NIAGARA FALLS, NEW YORK, A CORPORATION OF WEST VIRGINIA.

## METHOD OF TREATING MILL-SCALE.

1,127,163.

Specification of Letters Patent.

Patented Feb. 2, 1915.

No Drawing.

Application filed April 8, 1914. Serial No. 830,418.

To all whom it may concern:

Be it known that I, FREDERICK M. BECKET, a subject of the King of Great Britain, residing at Niagara Falls, in the county of Niagara and State of New York, have invented certain new and useful Improvements in Methods of Treating Mill-Scale, of which the following is a specification.

In my prior Patents Numbers 1,081,566 and 1,081,570, patented December 16, 1913, I have described certain processes applicable to the treatment of ores, concentrates, or like products, of the iron-tungstate type, to obtain therefrom tungsten or its alloys in which the ratio of tungsten to phosphorus,

expressed as  $\frac{W}{P}$ , is materially higher than

in the unreduced material.

20 The present invention relates to the application of processes of this kind to the oxidized material known as "high-speed mill-scale." This scale is produced in considerable quantities as a by-product in the manufacture of high-speed steel, and consists, essentially, of oxid compounds of iron and tungsten, usually with smaller proportions of chromium and vanadium and containing also considerable quantities of cobalt when 25 derived from the so-called cobalt steels. The metals are present in the scale in the form of oxid, but are not, in all cases at least, in their highest state of oxidation.

30 The following is the composition of a typical high-speed mill-scale:—

|            |                  |
|------------|------------------|
| Iron       | 57.66 per cent.  |
| Tungsten   | 12.25 "          |
| Chromium   | 3.28 "           |
| Vanadium   | 0.43 "           |
| Manganese  | 0.47 "           |
| Silicon    | 0.75 "           |
| Carbon     | 0.35 "           |
| Phosphorus | 0.015 to 0.030 " |

45 By smelting this scale with silicon as a reducing-agent, in an electric furnace and in accordance with the methods disclosed in my prior patents, it may be reduced to an alloy having approximately the composition 50 of the steel from which the scale was originally derived. For example, partial analyses of a mill-scale and the alloy obtained there-

from by known processes of silicon reduction, are as follows:

|          | Mill-scale. | Reduced alloy. |
|----------|-------------|----------------|
| Tungsten | 11.90       | 15.60          |
| Chromium | 2.90        | 3.40           |
| Vanadium | 0.49        | 0.43           |

The alloy so obtained is utilizable as such, 60 or, with appropriate additions, it is available for the manufacture of steels of modified composition. I have found, however, that such high-speed mill-scales usually contain a proportion of phosphorus which is 65 distinctly objectionable. Moreover, the product of direct reduction of the scale is comparatively low in tungsten: this of course necessitates the use of a relatively large proportion of the alloy in compounding 70 a given steel, from which it results that the phosphorus-content of the steel is not much less than that of the alloy. These difficulties are avoided by treating a mill-scale, before reduction, with an acid reagent 75 which serves the double purpose of removing iron, and thereby concentrating the tungsten-content, and of removing phos-

phorus, and thereby increasing the ratio  $\frac{W}{P}$ . 80

I have found that these mill-scales yield a large proportion of their iron, together with substantially all of their phosphorus, to acids, such as sulfuric acid, even in the 85 cold. In other words, the very high temperature to which they have been subjected in the course of their production has not resulted, as might be expected, in converting the iron into such an insoluble condition as 90 occurs when iron-tungstate ores are ignited or calcined. The process involving such acid-treatment of the mill-scale is claimed in my copending application Serial No. 830,417, 95 filed concurrently herewith.

According to the present modification of the invention, the mill-scale is subjected to a reducing operation before removing the phosphorus and concentrating its tungsten-contents. An illustrative example in accordance with the present invention is as follows:—The scale is ground to pass an eight-mesh screen and is mixed with about the theoretical proportion of charcoal or

other carbonaceous reducing-agent, calculated upon its contents of oxids of iron and tungsten. The proportion of charcoal used should be so restricted as to avoid substantial contamination of the reduced product by carbon, while effecting as nearly complete reduction of the iron and tungsten as may be practicable without such contamination. In other words, the proportion of carbon should be such that its elimination from the product is substantially complete, under which conditions the reduction is usually only approximately complete. This mixture is then heated in a suitable retort to a temperature of about 1,000° C., whereby reduction occurs below the melting-points of iron and tungsten. The reduced product is then subjected to treatment with an acid reagent under conditions to remove iron and phosphorus without material loss of tungsten. For example, it may be introduced into a bath of sulfuric acid of 1.2 to 1.4 specific gravity and digested for some hours, preferably with agitation. Following this digestion, the residue is washed to remove the soluble sulfate, dried, and smelted with a small proportion of silicon in the electric furnace. Silicon is added in approximately the theoretical proportions required for the reduction of such oxids as may have remained unreduced as a result of the first treatment, avoiding such excess of silicon as would yield a reduced product undesirably high in silicon. Lime or other flux may be added in proportion to form with the silica a suitable slag, as is well understood in this art.

According to this method, up to ninety per cent. of the total iron-content may be extracted without entailing material losses of tungsten. The resulting alloys may contain up to sixty-five per cent. of tungsten or more according to the amount of iron removed and are, for practical purposes, free from phosphorus.

I claim:

1. The herein-described method of preparing tungsten or its alloys from high-speed mill-scale containing tungsten, which consists in subjecting the scale to a reducing-operation at a temperature below the melting-point of the reduced product, extracting a portion of the iron and thereby concentrating the tungsten in such reduced product, and fusing the concentrate in an electric furnace.

2. The herein-described method of pre-

paring tungsten or its alloys from high-speed mill-scale containing tungsten, which consists in subjecting the scale to a reducing-operation at a temperature below the melting-point of the reduced product, extracting a portion of the iron and thereby concentrating the tungsten in such reduced product, and fusing the concentrate in an electric furnace in presence of a non-carbon reducing-agent.

3. The herein-described method of preparing tungsten or its alloys from high-speed mill-scale containing tungsten, which consists in subjecting the scale to a reducing-operation at a temperature below the melting-point of the reduced product, concentrating the tungsten in such reduced product and removing phosphorus therefrom, and fusing the concentrate in an electric furnace in presence of a non-carbon reducing-agent.

4. The herein-described method of preparing tungsten or its alloys from high-speed mill-scale containing tungsten, which consists in subjecting the scale to a reducing-operation at a temperature below the melting-point of the reduced product, concentrating the tungsten in such reduced product and removing phosphorus therefrom by an acid reagent, and fusing the concentrate in an electric furnace in presence of a non-carbon reducing-agent.

5. The herein-described method of preparing tungsten or its alloys from high-speed mill-scale containing tungsten, which consists in subjecting the scale to a reducing-operation at a temperature below the melting-point of the reduced product, concentrating the tungsten in such reduced product and removing phosphorus therefrom by an acid reagent, and fusing the resulting purified concentrate in an electric furnace in presence of silicon.

6. The method of preparing low-phosphorus tungsten or ferrotungsten from high-speed mill-scale, which consists in partially reducing said mill-scale, treating the reduced product to increase the ratio of tungsten to phosphorus, and thereafter completing the reduction.

In testimony whereof I affix my signature in presence of two witnesses.

FREDERICK M. BECKET.

Witnesses:

J. A. HOLLADAY,  
G. C. FURNESS.